

## UNITED STATES PATENT OFFICE.

OSKAR KALTWASSER, OF BERLIN, AND HERMANN KIRCHHOFF, OF DESSAU, IN ANHALT, GERMANY, ASSIGNORS TO I. G. FARBENINDUSTRIE AKTIENGESELLSCHAFT, OF FRANKFORT-ON-THE-MAIN, GERMANY.

## PROCESS FOR DYEING FURS, SKINS, HAIRS, FEATHERS, OR THE LIKE.

No Drawing. Application filed August 9, 1926, Serial No. 128,332, and in Germany July 10, 1925.

By the present invention furs, skins, hairs, feathers, or the like are dyed with the aid of the diamino-2-hydroxynaphthalene obtainable by dinitrating naphthalene-1-2-diazoxide, carefully treating the product with sodium sulphide and then reducing the nitrogroups, which product most probably is the 3,8-diamino-2-hydroxynaphthalene.

This compound is applied to the material 10 to be dyed in aqueous solution in the presence of an oxidizing agent at a moderate temperature.

The following example illustrates the invention without limiting it.

15 The well-washed skin is handled at 30° C. for 2 hours in a bath containing per liter 2 g. of diamino-2-hydroxynaphthalene hydrochlorate, 20 g. of hydrogen peroxide solution (of about 3 per cent strength) and 20 2 g. of ammonia of 25 per cent strength.

The skin is then rinsed, dried and finished as usual.

The dyeing on the unmordanted skin is brownish-gray. On a ferric mordant the dyeing is brownish-gray, on a chromic mordant it is dark-brown and on a cupric-mordant it is black-brown.

## What we claim is:

Process for dyeing furs, skins, hairs, and feathers, which comprises treating the material to be dyed, in the presence of an oxidizing agent, with a solution of the diamino-2-hydroxynaphthalene obtained by dinitrating naphthalene 1,2-diazoxide, carefully treating the product with sodium sulphide and then reducing the nitrogroups.

In testimony whereof we affix our signatures.

OSKAR KALTWASSER.  
HERMANN KIRCHHOFF.